

## UNITED STATES PATENT OFFICE.

HENRI BÉNIT, OF PARIS, FRANCE.

## ALUMINUM ALLOY OF HIGH RESISTANCE.

No Drawing. Application filed February 25, 1926, Serial No. 90,657, and in Germany February 19, 1925.

The subject of this invention is a new very light aluminum alloy distinguished by its high tensile strength and high-co-efficient of expansion. It is completely homogeneous and can be repeatedly melted without affecting its strength and expansion.

Experiments have shown that the best proportions are as follows:—

10 2 parts by weight of copper.  
0.37 parts by weight of nickel.  
0.27 parts by weight of tungsten.  
0.45 parts by weight of magnesium.  
96.91 parts by weight of aluminum.

15 The alloy can be conveniently produced in the following manner.

An alloy of copper, nickel and tungsten in the above proportions by weight is first produced. This alloy is introduced in a bath 20 of molten aluminum to which also magnesium is added in such a manner that the composition recited is obtained. The operations may be carried out in a different order or in a different manner so long as the alloy 25 produced has the composition indicated.

Test bars of the alloy described produced by casting in moulds have a tensile strength of about 22 kgs. per square mm. and in a length of 100 mm. have an expansion of 30 about 6%. After being forged stamped or rolled, test bars formed from the same alloy after being heated to incandescence and cooled in air show a tensile strength of about 20 kgs. per square mm. and 25% 35 expansion.

The composition of the aluminum alloy may be altered within certain limits so that the proportions may vary as follows:—

40 1.5 to 5 parts by weight of copper,  
0.3 to 3 parts by weight of nickel,  
0.2 to 2 parts by weight of tungsten,  
0.2 to 2 parts by weight of magnesium, and  
97.8 to 88 parts by weight of aluminum,

45 the quantity of the separate constituents varying between these limits so that, for example, 1.5 parts by weight of copper, 0.3 to 3 parts by weight of nickel and so on can be used.

50 There is thus produced a series of homogeneous and stable aluminum alloys of which

one can be used in molten condition while others again forged, stamped or rolled may be employed with advantage and the properties of which in substance are those of the 55 alloy first described.

Moreover these alloys possess after casting a tensile strength of 22 to 27 kgs. per square mm. with 5 to 10% expansion. By forging, stamping or rolling the tensile 60 strength is increased to 35 to 40 kgs. per square mm. with 20 to 25% expansion.

Thus, for example, an alloy formed of

2.5 parts by weight of copper, 65  
0.75 parts by weight of nickel,  
0.25 parts by weight of tungsten,  
0.50 parts by weight of magnesium, and  
96 parts by weight of aluminum,

was rolled after casting and produced test 70 bars which after being heated to incandescence and simply cooled in air showed a tensile strength of 36 kgs. per square mm. with 22% expansion.

These results were obtained with commercial aluminum containing 98-99% aluminum and 1-2% impurities. A slight improvement was found for instance with aluminum of 99.5% purity.

Having now particularly described and ascertained the nature of my said invention and in what manner the same is to be performed, I declare that what I claim is:—

1. A homogeneous and stable light aluminum alloy capable of being subjected to repeated melting without losing its characteristic properties, said alloy having substantially the following composition:—

2 parts by weight of copper, 90  
0.37 parts by weight of nickel,  
0.27 parts by weight of tungsten,  
0.45 parts by weight of magnesium,  
96.91 parts by weight of commercial aluminum,

95 with 2 to 0.5% impurities, cast test bars showing a tensile strength of 22 kgs. per square mm. with 6% expansion and test bars of the forged, stamped or rolled alloy showing a tensile strength of 30 kgs. per square 100 mm. with 23% expansion.

2. An aluminum alloy as claimed in claim

1, the composition of which is, however, modified and consisting of

- 1.5 to 5 parts by weight of copper,
  - 5 0.3 to 3 parts by weight of nickel,
  - 0.2 to 2 parts by weight of tungsten,
  - 0.2 to 2 parts by weight of magnesium,
  - 97.8 to 88 parts by weight of commercial aluminum,
- 10 with about 2 to 0.5% impurities, cast test

bars having a tensile strength of 22 to 27 kgs. per square mm. with 5 to 10% expansion and test bars of forged stamped or rolled alloy having a tensile strength of 35 to 40 kgs. per square mm. with 20 to 25% <sup>15</sup> expansion.

In witness whereof I have hereunto set my hand:

HENRI BÉNIT.